

## UNITED STATES PATENT OFFICE

1,968,797

SULPHURIC DERIVATIVE OF HIGHER  
ALCOHOLS

Heinrich Bertsch, Chemnitz, Germany

No Drawing. Application January 4, 1933, Serial  
No. 650,203. In Germany March 30, 1928

18 Claims. (Cl. 260—99.12)

This invention relates to soap-like products and to the manufacture of soaps, detergents, and the like, and to improvements in treatment liquids for use in the textile, leather, and allied industries. It is the primary object of the invention to produce new soap-like materials and other substances of this character having greater wetting, cleansing, dispersing, and foaming properties than the agents heretofore used.

Water-soluble sulphuric esters produced by the action of sulphuric acid on fatty materials, including both fatty acids and esters of fatty acids, containing double linkages and/or hydroxyl groups, are widely employed as wetting, cleansing, and dispersing agents in the textile and related industries. Thus a sulphuric acid ester of the hydroxy stearic acid may be produced by treating oleic acid with sulphuric acid, and a sulphuric acid ester of a dihydroxy stearic acid may be obtained by the treatment of ricinoleic acid with sulphuric acid. These agents are not entirely satisfactory, since sulphated fatty materials heretofore available contain carboxyl groups—either free or combined with alkali, depending upon the proportion of alkali used for neutralization after sulphation—and in consequence are capable of forming insoluble alkali earth salts. For instance, the difficultly soluble lime salts of these esters produce deleterious effects in the textile industry.

In accordance with the present invention, this defect is in large measure avoided if, instead of fatty acids or the esters of these acids, the corresponding alcohols obtained therefrom by replacement in effect of the carboxyl group whether free or combined with the  $\text{CH}_2\text{OH}$  group are treated with sulphuric acid or with other sulphating or sulphonating agent. Commercial fats are essentially mixed glycerides of the various higher fatty acids, and the higher alcohols obtainable therefrom are mixtures of alcohols of the general formula  $\text{C}_x\text{H}_y\text{—CH}_2\text{OH}$ . These mixtures consist predominantly of alcohols having 10 or more carbon atoms per molecule, corresponding to the molecular weight of the fatty acids, free or combined, contained in the natural fats and fatty oils and the other commercially available fatty materials derived therefrom. I have found that products soluble in water and valuable for use as wetting, cleansing, dispersing, and foaming agents can be obtained by treating such alcohols with sulphuric acid or with other sulphating or sulphonating agent. These alcohols may be referred to collectively as nor-

mal primary alcohols having more than eight carbon atoms to the molecule.

Thus the invention contemplates the conversion of the free or combined fatty acids of fatty materials, i. e. animal and vegetable fats and oils, and manufactured derivatives such as oleic acid or ethyl oleate, into the corresponding alcohols, and the treatment of these alcohols with a sulphating or sulphonating agent such as sulphuric acid. Usually it is also advisable to neutralize the reaction product with a base, for example sodium hydroxide or ammonia to form a water soluble soap-like salt, as is common practice in the case of sulphated fatty acids or sulphated fatty oils, such as Turkey red oil.

The precise nature of the method selected to convert the fatty material to the alcohol may be varied. For instance, a well-known method is that of Bouveault and Blanc, in accordance with which an alkyl ester of a fatty acid, e. g. an ethyl oleate, is reduced by sodium or other alkali metal and a lower aliphatic alcohol such as butyl alcohol, or the improved method described in my application for Letters Patent Serial No. 472,764 may be used. Numerous processes are known for preparing the alkyl esters from fats and fatty acids.

The Bouveault and Blanc process is of general application for the preparation of both unsaturated and saturated alcohols. For instance, by this process oleic alcohol ( $\text{C}_{17}\text{H}_{33}\text{—CH}_2\text{OH}$ ) may be prepared from esters of oleic acid ( $\text{C}_{17}\text{H}_{33}\text{COOH}$ ). An octodecyl alcohol ( $\text{C}_{17}\text{H}_{35}\text{—CH}_2\text{OH}$ ) may be formed from esters of stearic acid ( $\text{C}_{17}\text{H}_{35}\text{—COOH}$ ). Mixed saturated and unsaturated alcohols result when the unfractionated esters of the fatty acids of most natural fats, for example, tallow, are reduced according to the Bouveault and Blanc process.

An important example of a method for preparing predominantly saturated alcohols is catalytic hydrogenation of esters under high pressure, as described in the application for U. S. Letters Patent of Wilhelm Normann, Serial No. 510,326, filed January 21, 1931, and assigned to the assignee of the present application. This method may be applied directly to the conversion of the natural glycerides, such as coconut oil, to primary alcohols for use in accordance with the present invention.

Fatty alcohols obtained from the source described are next treated with a sulphating agent having water-binding properties. Ordinary concentrated sulphuric acid may be used, or stronger reagents such as anhydrous sulphuric acid,

chlorsulphonic acid, or fuming sulphuric acid. The principal reaction occurring is the formation of sulphuric esters, frequently called alkyl sulphuric acids, for instance, as follows:



In the case of an unsaturated alcohol, some addition of sulphuric acid at the double bond 10 also occurs, so that complete reaction of sulphuric acid with oleic alcohol would be according to the equation:



sulphuric ester of 1, 9-octadecanediol.

Unless a higher temperature is required to melt the alcohol, I prefer to effect sulphation in 20 the cold within the range of ordinary room temperature or lower, down to about 0° C. However, higher and lower temperatures can be used, and my invention is not restricted to a particular range of temperature of sulphation.

25 Under almost any practical condition of sulphation, there may be formed at least traces of sulphonic acids, the proportion of which may be increased by choice of sulphating medium and other conditions of reaction, for instance, by 30 high reaction temperatures and by the use of highly concentrated energetically acting reagents such as fuming sulphuric acid. While these are not my preferred reaction conditions, it should be understood that the sulphation products made in accordance with the present invention are not purely esters, but may contain also appreciable amounts of sulphonic acids or sulphonates. For convenience, the products resulting from the treatment with sulphuric acid or 40 other agent hereinbefore mentioned will be referred to generically as "sulphuric reaction products".

One method of sulphating which is of fairly 45 general application to different alcohol mixtures is to treat the alcohol just above its melting point with 100%–110% of the theoretical quantity of chlorsulphonic acid required according to the equation



The acid reaction products obtained as described above are preferably carefully neutralized, for instance, with sodium hydroxide. Neutralization should be carried out at relatively low 55 temperatures, preferably in a vessel fitted with a means for cooling. The resulting organic salts such as sodium lauryl sulphate may be separated from inorganic components such as sodium sulphate and sodium chloride by known methods, for instance, by dissolving in ethyl alcohol, decanting or filtering, and evaporating off the solvent. With or without this purification, the 60 products obtained are in general readily soluble in water, possess marked wetting, cleansing, dispersing, and foaming properties, and may be employed for manifold textile purposes. In a general way, they resemble the ordinary commercial 65 sulphuric esters of the fats and fatty acids, but are greatly superior in resistance to precipitation by lime salts and the other characteristic constituents of hard water.

The sulphated products of oleic alcohol are 70 particularly resistant to hardness and are high-

ly suitable for use in the textile and related industries.

Likewise a high resistance to the action of hard water is shown by the sulphated products of lauryl alcohol, which is the principal constituent of the mixed alcohols obtained by reduction of coconut, palm kernel and similar oils, or by reduction of the alkyl esters or the free fatty acids of these oils. Sulphated alcohols of this class have remarkable cleansing and foaming properties, and are valuable as soap substitutes, especially for use in hard water.

The sulphuric reaction products derived from lauryl alcohol, especially the esters and salts thereof, are also found to be particularly effective in the textile industry. Thus when starting from the fatty alcohols made from free fatty acids of the coconut oil or palm seed oil in a manner known per se by esterifying the fatty acids of the same with lower aliphatic alcohols and reducing the mixture of esters by means of sodium, it is advantageous to distill the reduction product and to use only the first 50% to 60% of the distillate. The product thus obtained consists mainly of lauryl alcohol, the somewhat less suitable higher fractions which contain principally myristyl alcohol and octadecyl alcohol being substantially eliminated. It should be understood, however, that the presence of the sulphuric derivatives of lower or higher alcohols, such as 105 of myristyl alcohol with the lauryl alcohol derivatives does not materially decrease the efficiency of the final product.

Various other higher alcohols may be produced and converted into wetting and cleansing 110 agents, substantially according to the procedure indicated in the above examples, for instance the following:

Alcohols obtained by catalytic hydrogenation 115 of the free fatty acids of coconut oil and comprising mainly lauric alcohol, myristic alcohol, cetyl alcohol, and stearic alcohol or the single alcohols separated from each other by fractional distillation.

Alcohols obtained by catalytic hydrogenation 120 of palm kernel oil or of the free fatty acids of palm kernel oil comprising similar constituents as the alcohols obtained from coconut oil.

Alcohols obtained by saponification of spermaceti, sperm oil, beeswax and distillation according to Axelrad and Hochstadter (U. S. A. Patent 1,290,870).

Linoleic alcohol obtained by reduction of linoleic acid by means of sodium and ethyl alcohol.

Alcohols obtained by catalytic reduction of tallow or the free fatty acids of tallow.

Alcohols obtained by catalytic hydrogenation of the free fatty acids of coconut oil.

Alcohols obtained by catalytic hydrogenation of 135 the free fatty acids of palm kernel oil.

Alcohols obtained by reducing olive oil by means of metallic sodium and butyl alcohol.

Alcohols obtained by reducing the ethyl esters of tallow fatty acids by means of metallic sodium 140 and butyl alcohol.

Alcohols obtained by catalytic hydrogenation of the ethyl ester of commercial stearic acid.

Ricinoleic alcohol obtained by reduction of 145 ricinoleic acid by means of sodium and ethyl alcohol.

The following examples are given to illustrate the manner in which the process may be carried out:

80

85

90

95

100

105

110

115

120

125

130

135

140

145

150

**Example 1**

100 kgs. of a mixture of fatty alcohols mainly consisting of lauryl alcohol, and obtained from coconut oil by esterification of the fatty acids with ethyl alcohol, reduction of the ethyl ester, distillation of the product of the reduction and collection of the first 50% to 60% of the distillate, are heated to melting temperature about 30° C. and treated at this temperature with 50 kgs. of chlorsulphonic acid.

The foregoing reaction may be represented by the following formula:



100 kgs. of pure lauryl alcohol would require for best results a higher proportion of chlorsulphonic acid about 60 kgs.

**Example 2**

100 kgs. of the same mixture of fatty alcohols is sulphonated with 70 kgs. of fuming sulphuric acid 10% SO<sub>3</sub> at the temperature of 50° C.

The products of the reaction are directly neutralized by means of soda lye and separated by known methods from inorganic components such as sodium sulphate or sodium chloride.

**Example 3**

100 kgs. of a mixture of fatty alcohols obtained by catalytic reduction of spermaceti with hydrogen and a copper catalyst at a temperature between 300 and 350° C. and a pressure of 150-200 atmospheres until the acid number has wholly disappeared, are sulphonated at a temperature of 35° C. with 60 kgs. of chloro-sulphonic acid. The product is poured in 200 kgs. of ice water and is then neutralized by means of a potassium hydroxide solution. There results a white paste readily soluble in water.

The reactions occurring can be represented by the following equations:

**Example 4**

100 kgs. of oleic alcohol are sulphated at 25° C. with 80 kgs. of concentrated sulphuric acid. The mixture is poured into 150 kgs. of ice water and is neutralized by means of piperidine.

The reaction may be represented by the following equations:

**Example 5**

100 kgs. of the mixture of unsaturated and saturated fatty alcohols obtained by reduction of coconut oil by means of an alkali metal and butyl alcohol, adding water, separating the resulting watery alkali hydroxide solution and removing the butyl alcohol by distillation, are treated with 80 kgs. of chlorsulphonic acid at 35° C. The product is worked up as described in Example 3, neutralized with sodium hydroxide solution to form a white, readily water-soluble paste.

**Example 6**

100 kgs. of ricinoleic alcohol obtained by reduction of ricinoleic acid by means of sodium and amyl alcohol, adding water, separating the watery alkali hydroxide solution and removing the amyl alcohol by distillation are treated with 150 kgs. of concentrated sulphuric acid at a temperature between 10 and 20° C. The product is worked up as described in Example 3 and neutralized by means of equal parts of sodium hydroxide solution and potassium hydroxide solution. An oily product readily soluble in water is obtained. The main reaction is probably represented by the following equation:



Besides this reaction there may be also a reaction of only two or only one of the free groups (two hydroxyl groups and one double linkage) capable of reaction with sulphating means. These reactions yield for example the following products

**Example 7**

100 kgs. of stearic alcohol are treated at 40-50° C. with 50 kgs. of chlorsulphonic acid. The product is worked up as described in Example 3. A white paste is obtained. The reaction can be represented by the following formula:

**Example 8**

100 kgs. of a mixture of the alcohols obtained by saponification of spermaceti oil by means of caustic lime and distillation of the saponification product according to U. S. A. Patent 1,290,870, said alcohols having an iodine number of about 50 and consisting mainly of cetyl alcohol and oleic alcohol, are mixed with 100 kgs. of concentrated sulphuric acid at 40° C. The mass is then poured into 200 kgs. of ice water. The mixture is neutralized by adding sodium hydroxide solution of 28° Bé. The resulting solution containing 15-20% calculated on free fatty alcohol, is introduced in a spraying dryer of the Krause system and dried at a temperature between 75-80° C., the temperature of the hot air entering at the bottom of dryer being about 170° C.

Before or after the drying operation such quantities of Glauber's salt may be added to the solution or to the dried product respectively, that the final product contains for example 35% calculated on free fatty alcohol.

**Example 9**

100 kgs. of linoleic alcohol obtained by reduction of linoleic acid by means of an alkali metal and ethyl alcohol in a manner known per se, are dissolved in 50 kgs. of water free ethyl ether and treated with 200 kgs. of concentrated sulphuric acid at a temperature between 0 and 5° C. for several hours. The product is mixed with 300 kgs. chopped ice and 50 kgs. ethyl ether, washed with saturated Glauber's salt solution and neutralized by means of triethanolamine.

The reaction is probably represented by the following equation:



5 Besides the esterification of the  $\text{CH}_2\text{OH}$  group also  
addition of sulphuric acid to one or both of the  
double linkages may occur.

10 The following fatty materials have been found  
particularly suitable for conversion to alcohols  
and thence to sulphuric acid derivatives: tallow,  
lard, whale oil, coconut oil, palm kernel oil, palm  
oil, olive oil, castor oil, linseed oil, tall oil, technical  
stearic acid, technical oleic acid and ricinoleic  
acid, palmitic acid, tallow fatty acids, Japan  
wax, spermaceti, sperm oil, beeswax, Montan  
wax, methyl, ethyl, propyl and butyl esters of  
technical fatty acid mixtures such as stearic acids,  
oleic acids, tallow fatty acids, linseed oil fatty  
acids and whale oil fatty acids.

20 The present invention is disclosed in my prior  
applications Serial Nos. 350,135, filed March 26,  
1929, and 433,815 filed March 6, 1930, of which  
the present application is a continuation in part.

25 It is to be understood that this invention is not  
limited to the specific embodiments hereinbefore  
disclosed, but that it includes all modifications  
as to procedure and all equivalent materials com-  
ing within the terms of the claims and the scope  
or the tenor of the specification.

30 Having thus described the invention, what is  
claimed as new and desired to be secured by Let-  
ters Patent is:

35 1. In the manufacture of soap-like materials,  
the combined steps of converting the carboxyl  
groups of a fatty material to primary alcohol  
groups and then reacting the resulting alcohols  
with a sulphonating agent.

40 2. A soap-like material comprising essentially  
salts of alkyl sulphuric acids derived from primary  
alcohols resulting from the reduction of the fatty  
acid radicals contained in fatty material.

45 3. A wetting and cleansing agent comprising  
essentially water-soluble sulphuric esters of alco-  
hols obtained by sulphation of fatty material  
from which carboxyl groups, including combined  
carboxyl groups, are eliminated.

50 4. A wetting and cleansing agent comprising  
essentially a water-soluble sulphation product of  
primary alcohols resulting from the reduction of  
the fatty acid radicals contained in fatty material.

55 5. In the production of wetting and cleansing  
agents, the combined steps of converting the car-  
boxyl groups of a fatty material to primary alcohol  
groups and then sulphating.

60 6. In the production of wetting and cleansing  
agents, the combined steps of reducing the esters  
of fatty and oily acids having more than 8 carbon  
atoms to the corresponding higher alcohols and  
thereafter sulphating the resulting alcohols.

65 7. In the production of wetting and cleansing  
agents, the combined steps of reducing the esters  
of fatty acids having more than 8 carbon atoms

to the corresponding higher alcohols by treat-  
ment with an alkali metal and a lower alcohol,  
and thereafter sulphating the resulting higher  
alcohols.

8. The process of manufacturing wetting and  
cleansing agents which comprises reducing a fatty  
material to form higher alcohols corresponding  
to the fatty acid radicals contained therein, sul-  
phating said higher alcohols to form alkyl sul-  
phuric acids and neutralizing with a base to yield  
water-soluble salts of said alkyl sulphuric acids. 80

85 9. A composition of matter having soap-like  
properties consisting essentially of sulphuric esters  
of aliphatic alcohols having more than 8 carbon  
atoms obtained from fatty material by eliminat- 90  
ing carboxyl groups from the carboxyl containing  
constituents.

95 10. Sulphated mixture of primary alcohols ob-  
tained by conversion of fatty materials contain-  
ing fatty acids including combined fatty acids  
having more than 8 carbon atoms in the chain. 95

100 11. A wetting and cleansing agent comprising  
a sulphation product of an unsaturated alcohol  
obtained by reducing an unsaturated fatty mate-  
rial having more than 8 carbon atoms. 100

105 12. The process of producing wetting and  
cleansing agents composed of alcohol sulphate  
salts having more than 8 carbon atoms comprising  
producing alcohols from a fatty material contain-  
ing fatty acid radicals of more than 8 carbon  
atoms, sulphating said alcohols at a temperature  
sufficiently low to produce principally sulphates  
and in the absence of organic solvents of said  
alcohols, and then neutralizing the reaction prod-  
ucts to form the salts of the sulphated alcohols. 110

115 13. The process of producing alcohol sulphates  
having from 12 to 18 carbon atoms inclusive, com-  
prising producing alcohols from a fatty material  
containing fatty acid radicals of the above men-  
tioned number of carbon atoms, and sulphating  
said alcohols at a temperature sufficiently low to  
produce substantially only sulphates and in the  
absence of organic solvents of said alcohols. 115

120 14. The product produced by the process de-  
scribed in claim 12. 120

125 15. The product produced by the process de-  
scribed in claim 13. 125

16. Sulphuric ester of primary stearyl alcohol.

17. A composition of matter having soap-like  
properties consisting essentially of sulphuric  
esters of normal primary aliphatic alcohols hav-  
ing from 12 to 18 carbon atoms inclusive, obtained  
from fatty material by eliminating carboxyl  
groups from the carboxyl containing constituents. 125

130 18. A soap-like material comprising essentially  
salts of acids of the group consisting of alkyl  
sulphuric acids and alkyl sulphonic acids derived  
from primary alcohols resulting from the reduc-  
tion of the fatty acid radicals contained in fatty  
material. 130

HEINRICH BERTSCH. 135